# EUROPEAN PATENT APPLICATION

(11) **EP 0 306 639 A1**
(43) Date of publication of application: **15.03.1989**
(21) Application number: 88109875.0
(22) Date of filing: 21.06.1988
(51) Int. Cl.: D21D 3/00, D21H 5/00

(54) **Process for the manufacture of magnetic paper and paper thereof**

(30) Priority: 11.09.1987 IT 2188487
(71) Applicant: CARTARIA FAVINI S.r.l., Rossano Veneto Vicenza (IT)
(72) Inventor: Nicolucci, Clemente, Padova (IT)

(57) **Abstract**

A process is described for the manufacture of magnetic paper by directly operating in the production step in a continuous papermaking machine.

## Description

The present invention relates to a process for the manufacture of magnetic paper and to the paper thus obtained.

The following description particularly relates to the paper but the disclosed process is also suitable for the production of Bristol board having magnetic property which is included in the scope of the present invention.

In the last years an exceptional development has been attained in the recording systems of music of sounds and of electronic data for computer processing.

Magnetic tapes are normally used consisting of a polymeric film support, e.g. of polyester type, coated by a thin layer of a suitable adhesive dispersion composition formed by small particles of gamma iron oxide crystals possibly modified with other types of metals or oxides.

Iron oxide is permanently magnetized by passing the obtained tape through a magnetic head (recording head) which is orienting the oxide crystals.

The magnetic tape recording is widely used for preparing the magnetic badges for personal identification which are used for financial or banking services tele-controlled through electronic computers.

The normally used magnetic badges are consisting of polymeric material support, which is sufficiently tough for avoiding the accidental bending whereon a thin layer of a normal magnetic tape is sized or a magnetic link is deposited.

The magnetic effect is also widely used in the anti-thief labels for goods in the stores, in the magnetic keys, in magnetic boards or toys, in the locking systems for furniture and so on.

It has now been found that it is possible to directly magnetize the common cellulose and/or other natural and/or synthetic fibers paper thus giving to it the property of recording magnetic signals as the polyester tapes sold for such a target.

According to a fundamental aspect of the present invention, a powderized metallic oxide permanently magnetizable of the type normally used for magnetic tapes is mixed with the cellulose (or other fibers) pulp for paper. Gamma crystalline form of iron oxide is particularly suitable to this purpose.

Other suitable magnetizable materials are chromium oxides, silicon-iron alloys, nickel-iron alloys (permalloy), aluminium-nickel-cobalt-copper alloys (alnico alloys), samarium-cobalt alloys, soft ferrites, hard ferrites.

It is obviously possible to obtain a large range of magnetic properties of the final paper depending on the type and on the amount of magnetizable material used for its manufacture.

According to a fundamental aspect of the present invention, the magnetizable material in powder form of from 0.1 to 10 micrometer is added to the fibers paper pulp in substitution and/or in addition of the normally used pigments like talc, caolin, titanium dioxide.

According to the present invention, from 2% up to 30% by weight of magnetizable material is typically added to the paper for making it magnetizable.

According to another fundamental aspect of the process of the invention the paper leaving the continuous papermaking machine is carefully smoothed either directly in the machine either by further treatment of the finished paper sheet. The paper sheet is smoothed by passing through the rollers of a calender at the same temperature which is used for the common paper, i.e. between 20 and 80 degrees C, and at a pressure of from 0.2 to 5 bar.

According to another typical embodiment of the invention's process, the magnetizable material is applied to the surface of the paper web during the coating step, by mixing them with traditional binders and by substituting or by adding to the usual mineral charges.

Useful binders for this form of embodiment of the invention are the starch derivatives, the hydroxyethylcellulose, the carboxymethylcellulose, the latices of synthetic resins particularly of vynilic and/or acrylic resins, the polyvynil alcohols, the aqueous emulsions of acetovynil polymers. In these embodiments the weight ratio of magnetizable material to the other additives is between 0.5:1 and 4.5:1 and the amount of added magnetizable material is between 0.1 and 20% by weight in respect of paper.

If the paper according to the invention is prepared for use as recording medium, it behaves as a normal recording magnetic tape and can be recorded by an usual recording apparatus without any need of modifying the recording head, provided for the paper is cutted in strips of suitable height to be compatible with the said head.

It is evident the advantage of disposing of such an usual support as the paper having the property of being magnetizable and of consequence directly usable to said end use without any need of further applying the other substances in successive steps following the preparation of the support itself.

Between the most interesting uses of the magnetizable paper of the invention, we can list the manufacture of small insertion for talking or musical toys, adhesive strips for goods coding readable by magnetic apparatus, magnetic badges of Bristol board of a suitable weight, optionally plastified, anti-thief labels for goods in the stores, magnetic boards or toys, locking systems for furniture, magnetic masking tapes for car painting.

The following examples are better illustrating the present invention without willing to limit it.

### EXAMPLE 1

A continuous papermaking machine having a capacity of 4,000 kg/hr of paper was employed to make a pulp for white paper formed by 70% of birch wood sulfite cellulose and by 30% of conifer wood sulfite cellulose. 20% by wt. in respect of cellulose of gamma iron oxide was added to, the oxide being commercialized under the trade name Magnox - B 350 by Magnox Pulaski Corp.

The pulp was traditionally refined up to 30 - 40 Schopper Riegler degrees. 0.5% by wt. in respect of cellulose of the retention aid commercialized by Sandoz under the trade name Cartaretin F was added to. The dry content of the pulp was 5% by weight.

The speed of the web leaving the machine was adjusted at 200 m/min. The web leaving the machine was calendered through a Vari-Nip calender normally in use for smoothing the paper for printing. The obtained paper was black. Strips having a height of 4 mm were checked in a tape recorder for recording and playing back sounds and voices with very good performances even after several passages through the recorder.

### EXAMPLE 2

Ammonium stearate 400 g and then hydroxy - ethyl -cellulose 6 kg were added to water 150 1 under stirring up to complete dissolution of the stearate.

Then magnetic iron oxide (commercialized by Bayer as code 5055) 40 kg was added to and the slurry was stirred for 2 hrs then a fluidizer (commercialized by Gaf as Gafac RH 710) 250 g was added to. The slurry was filtered through a 3 micrometer mesh sieve and used as coating in the size press.

The speed web of the paper machine was adjusted to 40 m/min so to produce 600 g/hr of a Bristol board of 160 g/sq. m of weight. The width of the web of the paper machine was 150 cm.

The obtained coating was applied to one side of the Bristol board in an amount of 5 g/sq.m. Of course, it was possible to coat both the Bristol board sides without any further difficulty.

## Claims

1. Process for the manufacture of magnetic paper characterised by adding a powderized magnetizable material to the pulp paper fed to the coater or to the size press in the papermaking machine.

2. Process as claimed in claim 1 characterized in that the powderized magnetizable material has a size of from 0.1 to 10 micrometers.

3. Process as claimed in claim 1 characterized in that the powderized magnetizable material is iron oxide in the gamma crystalline form.

4. Process as claimed in claim 1 characterized in that the powderized magnetizable material is added to the cellulose pulp paper in substitution and/or addition of commonly used pigments as talc, caolin, titanium dioxide.

5. Process as claimed in claim 1 characterized in that the amount of powderized magnetizable material added to the paper is of from 2% to 30% by weight in respect of paper.

6. Process as claimed in claim 1 characterized in that the paper leaving the paper machine is smoothed by passing through the rollers of a calender at a temperature between 20 and 80 degrees C and at a pressure of from 0.2 to 5 bar.

7. Process as claimed in claim 1 characterized in that the powderized magnetizable material is applied to the surface of the paper web during the coating step by mixing with traditional binders and by substituting or by adding to the usual mineral charges.

8. Process as claimed in claim 7 characterized in that the binders are selected between the starch derivatives, the hydroxy - ethyl - cellulose, the carboxy - methyl - cellulose, the latices of synthetic resins particularly of vynilic and/or arcylic resins, the polyvynil alcohols, the aqueous emulsions of acetovynil polymers.

9. Process as claimed in claim 7 characterized in that the weight ratio of powderized magnetizable material to the other additives is between 0.5:1 and 4.5:1 and its amount is between 0.1 and 20% by weight in respect of paper.

10. Magnetic paper obtained by addition of powderized magnetizable material to the pulp paper in the continuous papermaking machine.
